# EUROPEAN PATENT SPECIFICATION

(11) **EP 0 638 116 B1**
(45) Date of publication and mention of the grant of the patent: **02.06.1999**
(21) Application number: 90916328.9
(22) Date of filing: 30.10.1990
(51) Int. Cl.: C10M 105/12

(54) **NON-STAINING SOLID LUBRICANTS**
NICHTVERSCHMUTZENDE FESTE SCHMIERMITTEL
LUBRIFIANTS SOLIDES NON TACHANTS

(30) Priority: 31.10.1989 GB 8924457
(43) Date of publication of application: 15.02.1995
(73) Proprietor: ALCAN INTERNATIONAL LIMITED, Montreal Quebec H3A 3G2 (CA)
(72) Inventor: FOSTER, Mark, Howard, Oxfordshire OX16 9TQ (GB); PARGETER, Christopher, Oxfordshire OX16 7DN (GB)
(74) Representative: Wilkinson, Stephen John
(86) International application number: GB9001659
(87) International publication number: WO9106619

(56) References cited:
- EP-A- 0 192 329
- US-A- 3 765 955
- US-A- 3 899 433

## Description

The present invention relates to non-staining solid lubricants suitable for use in metal working operations, for instance in cold-rolling, drawing or extrusion of metals, especially aluminium.

Lubricants, usually liquid lubricants, are used in metal working operations to reduce friction between the surface of metal being worked and a surface of the apparatus carrying out the operation. A liquid lubricant reduces friction by separating the two surfaces with a thin fluid film having little resistance to shear. In many metal working operations the pressure between a surface of the metal being worked and a surface of the apparatus is so great that the fluid film of a liquid lubricant may be squeezed out so allowing actual metal-to-metal contact with the result that excessive damage to the surfaces may occur. Solid film lubricants having much greater load bearing properties have been developed to overcome this and other disadvantages associated with liquid lubricants.

In addition to its lubrication characteristics, a lubricant may be expected to fulfil certain other requirements if it is to be useful industrially. For instance, it should be easy to apply and easy to remove, it should afford some protection to the metal surface during handling and storage, it should present no health hazard to persons coming into contact with it and, obviously, should be inert to the surfaces with which it comes into contact. Many lubricants produce severe stains on the surface of the metal during annealing thereof. It is, therefore, highly desirable to avoid such staining by using a lubricant having the properties demanded by the particular conditions under which the lubricated metal is to be worked and which is also non-staining.

The present invention is based on the discovery that a solid film of one or more saturated aliphatic monohydric alcohols having from 14 to 18 carbon atoms provided on the surface of the metal being worked has good lubrication characteristics under cold-working conditions and can be removed by heating to leave substantially no stain on the metal surface.

The present invention provides a method of cold forming a metal workpiece comprising providing on the surface of the workpiece to be subjected to forming a film of a lubricant, subjecting the workpiece to a forming operation and removing the film of lubricant from the metal surface characterised in that the lubricant film comprises a solid film of a saturated aliphatic monohydric alcohol having from 14 to 18 carbon atoms and in that the lubricant film is removed from the metal surface without causing staining by the application of heat thereto.

The present invention further provides the use of a saturated aliphatic monohydric alcohol having from 14 to 18 carbon atoms as a solid lubricant in the cold working of a metal workpiece removed from the surface of the metal by heating without staining. The present invention also provides the use of a composition comprising a solution of a saturated aliphatic monohydric alcohol having from 14 to 18 carbon atoms in an inert volatile organic solid as a lubricant film-forming agent in the cold working of a metal workpiece to form a film of solid 14-18 C saturated aliphatic monohydric alcohol lubricant on the workpiece surface removed from the metal surface by heating without staining.

According to the invention, use is made of a saturated aliphatic monohydric alcohol having from 14 to 18 carbon atoms. Such alcohols have good lubricating and load-supporting properties, are solid at room temperatures (20-25°C) and may be, at worst, only slightly staining or, at best, totally non-staining. Examples of these alcohols include myristyl alcohol, cetyl alcohol and stearyl alcohol. Commercial purity compounds may be used and these generally contain proportions of higher and/or lower homologues as impurities. Cetyl alcohol (hexadecanol) is highly preferred for use in the present invention in view of its melting point (∼49°C) and because of its excellent non-staining property.

Typically, the 14-18C saturated aliphatic monohydric alcohol lubricant is applied to the surface of the metal workpiece by dip coating the workpiece in a solution of the alcohol lubricant in an inert volatile organic solvent. After removal of the volatile solvent by evaporation a film of the solid alcohol remains on the surface of the workpiece. It is possible that the film obtained in this way may not be of uniform thickness; the deposited alcohol lubricant being thicker in some regions than in other regions of the surface of the workpiece. We have observed, however, that in such cases where the thickness of the deposited film of solid alcohol is non-uniform the film flows at the point where pressure is applied to the workpiece during working thereof, e.g. at the die in a metal drawing operation or at the press platen in a metal pressing operation, with the result that the workpiece becomes evenly covered at the point of working.

To form the lubricant coating composition, the 14-18C saturated aliphatic monohydric alcohol is dissolved in an inert volatile organic solvent. Generally, any organic solvent for the alcohol which is liquid at normal room temperature but which evaporates at a temperature just above that and which is inert to both the alcohol and the metal surface may be used. Examples of suitable solvents include diethyl ether, methanol and benzene and chlorinated hydrocarbons, such as trichloroethylene and 1,1,1-trichloroethane. The concentration of the 14-18C alcohol in the volatile organic solvent is not critical and, in principle, any concentration up to the solubility limit of the particular solvent may be used. Typically, the concentration of alcohol in the organic solvent will be about 10% by weight.

According to the present invention, it is possible to incorporate certain amounts of other substances in the lubricating film of 14-18C saturated aliphatic monohydric alcohol in order to modify the properties of the film. For instance, a liquid polybutene may be incorporated in an amount of up to 10% by weight of the total weight of the lubricant composition (excluding solvent) to modify the film properties of the lubricant on the surface of the workpiece and the flow characteristics of the lubricant film during the deformation without causing staining of the metal surface on annealing. The use of the liquid polybutene tends to soften any film containing it and the 14-18 saturated aliphatic monohydric alcohol and, therefore, if more than 10% by weight of the liquid polybutene is used the lubricant film obtained on the surface of the workpiece may become tacky and rather unstable. Any liquid polybutene may be used according to this embodiment of the invention. Liquid polybutenes are available commercially under the name Hyvis ("Hyvis is a registered trademark), for example Hyvis 200, having a molecular mass (number average) of 2400 and a Kinematic viscosity of 4300 cSt at 98.9°C.

The non-staining solid lubricant according to the present invention may contain a small amount of a solid or semiliquid (e.g. gelatinous) alkane species or mixture of alkane species which does not leave a staining residue on annealing, for example petroleum jelly (petrolatum), to modify the film properties of the lubricant. Such an alkane-based film modifier may be used together with or as an alternative to the liquid polybutene mentioned above. Generally, any alkane-based film modifier if used will be used in an amount such that the combined weight of alkane-based film modifier and any liquid polybutene does not represent more than 10% of the weight of the total lubricant composition (excluding solvent). We have further found that the incorporation of an (liquid) ester, e.g. butyl stearate, methyl laurate or methyl myristate, in the 14-18C saturated aliphatic monohydric alcohol lubricant film tends to aid the production of a uniform film and also tends to soften the film. This tendency to soften the film is an additional advantage in the case where the lubricant also contains a polybutene additive since it makes it easier for the polybutene-containing lubricant to be removed from surfaces (including hands). If used, the ester may be used in an amount not exceeding 10% by weight based on the total weight of the lubricant (excluding solvent) and would be incorporated as an alternative to an equivalent amount of liquid polybutene. We refer, however, not to use more than about 1% by weight of the ester.

The solid lubricant, after evaporation of the volatile carrier solvent, forms a tenaceous film on the surface of a metal workpiece. A typical lubricant coverage would be less than about 10gm⁻². Preferably, however, the lubricant solution will be applied to a metal surface to provide about 5g of solid lubricant per square metre of surface.

After deformation etc. of the workpiece the solid film lubricant does not require removal prior to annealing the metal since the component(s) of the solid lubricant, i.e. the alcohol and any optionally present polybutene, petroleum jelly and/or butyl stearate, will evaporate from or decompose on the metal surface cleanly without staining.

### EXAMPLES

### Example 1

An aluminium tube was dipped in a 10% w/w solution of cetyl alcohol in trichloroethylene and then allowed to dry. The coated tube was passed four times through a drawing machine. After each pass, the tube was annealed by heating to 400°C, with no prior degreasing and no staining and then re-dipped in the cetyl alcohol solution. The following Table 1 shows the outside and inside diameters of the tube, the percentage reduction in the cross sectional area, and the length of the tube after each pass. The reductions are set by the size of the die used, which is why they are variable. However, the final reduction of 23% is excellent and the tube after the final pass showed no surface staining.

**Table 1**

| | Outside diameter | Inside diameter | % Reduction | Length |
|---|---|---|---|---|
| | (mm) | (mm) | | (m) |
| Initial dimensions of tube | 293.0 | 275.4 | - | 3 |
| After 1st pass | 287.3 | 272.6 | 21 | 3.6 |
| After 2nd pass | 283 | 269.9 | 12.4 | 4.2 |
| After 3rd pass | 278 | 267.2 | 19 | 5.2 |
| After 4th pass | 273.8 | 265.4 | 23 | 6.8 |

### Example 2

A series of disc compression tests was carried out using various lubricants. In each case, an aluminium disc having a diameter of 32mm and a thickness of 5mm was dipped into a solution of the lubricant under test in a volatile organic solvent so that both the upper and the lower surfaces of the disc were coated with the lubricant solution. The coated disc was then left until the organic solvent had evaporated to leave a coating of lubricant on the aluminium surface. Each disc was subjected to pressing at 5.6 x 10⁷ kg m⁻² over a period of 30 seconds and the thickness of the disc was then measured. The test was carried out 5 times for each lubricant and the mean reduction (%) was calculated. Each lubricated disc was annealed at 400°C and checked for any staining. The results are shown below in Table 2.

**Table 2**

| Lubricant | Reduction (%) | | Staining of Metal Surface on annealing (400°C) |
|---|---|---|---|
| | Mean | Std.deviation | |
| *'Batoyl' | 49.9 | 0.77 | heavy dark stain |
| *'Silkolene' | 48.4 | 0.33 | heavy dark stain |
| 100% cetyl alcohol | 56.7 | 0.55 | none |
| 90% cetyl alcohol | 60.9 | 0.61 | none |
| 10% petroleum jelly | | | |
| 75% cetyl alcohol | 59.5 | 0.62 | none |
| 25% petroleum jelly | | | |

| | | | |
|---|---|---|---|
| * 'Batoyl' and 'Silkolene' are proprietory solid film lubricants based on a heavy oil containing extreme pressure additives. | | | |

## Claims

1. A method of cold working a metal workpiece comprising providing on the surface of the workpiece to be subjected to forming a film of a lubricant, subjecting the workpiece to a forming operation and removing the film of lubricant from the metal surface characterised in that the lubricant film comprises a solid film of a saturated aliphatic monohydric alcohol having from 14 to 18 carbon atoms and in that the lubricant film is removed from the metal surface without causing staining by the application of heat thereto.

2. A method according to claim 1, wherein the solid lubricant film is caused to flow on the metal surface at a point where pressure, due to the forming operation, is applied.

3. A method according to either claim 1 or claim 2, wherein the saturated aliphatic monohydric alcohol is cetyl alcohol.

4. A method according to any one of claims 1 to 3, wherein the lubricant further contains from 1 to 10% by weight of the total weight of the lubricant of a polybutene, petroleum jelly or butyl stearate.

5. The use of a saturated aliphatic monohydric alcohol having from 14 to 18 carbon atoms as a solid lubricant in the cold working of a metal workpiece removed from the surface of the metal by heating without staining.

6. The use according to claim 5, wherein the saturated aliphatic monohydric alcohol is cetyl alcohol.

7. The use according to either claim 5 or claim 6, wherein the lubricant also contains from 1 to 10% by weight of the total weight of the lubricant of a polybutene, petroleum jelly or butyl stearate.

8. The use of a composition comprising a solution of a saturated aliphatic monohydric alcohol having from 14 to 18 carbon atoms in an inert volatile organic solid as a lubricant film-forming agent in the cold working of a metal workpiece to form a film of solid 14-18 C saturated aliphatic monohydric alcohol lubricant on the workpiece surface removed from the metal surface by heating without staining.

9. The use according to claim 8, wherein the saturated aliphatic monohydric alcohol is cetyl alcohol.

10. The use according to either claim 8 or claim 9, wherein the inert volatile organic solvent is selected from trichloroethylene and 1,1,1 -trichloroethane.

11. The use according to any one of claims 8 to 10, wherein the solution contains about 10% by weight of the saturated aliphatic monohydric alcohol.

12. The use according to any one of claims 8 to 11, wherein the solution additionally contains a material selected from a polybutene, petroleum jelly and butyl stearate in an amount of from 1 to 10% by weight based on the combined weight of the saturated aliphatic monohydric alcohol and the said material.

13. The use according to any one of claims 5 to 12, wherein the metal workpiece is formed of aluminium or an aluminium alloy.

14. The use according to any one of claims 5 to 13, wherein a metal workpiece in the form of a tube is selected to a cold drawing operation.

## Patentansprüche

1. Verfahren zur Kaltbearbeitung eines Metallwerkstücks, umfassend das Bereitstellen eines Gleitmittelfilmes auf der Oberfläche des Werkstücks, welches einem Formen zu unterwerfen ist, Unterwerfen des Werkstücks einer Umformung und Entfernen des Gleitmittelfilmes von der Metalloberfläche, dadurch gekennzeichnet, dass der Gleitmittelfilm einen festen Film eines gesättigten aliphatischen Monoalkohols mit 14 bis 18 Kohlenstoffatomen umfasst und dass der Gleitmittelfilm von der Metalloberfläche ohne Fleckenbildung durch die Anwendung von Hitze hierauf entfernt wird.

2. Verfahren gemäss Anspruch 1, wobei der feste Gleitmittelfilm auf der Metalloberfläche an einem Punkt, an dem Druck aufgrund der Umformung aufgebracht wird, zum Fliessen gebracht wird.

3. Verfahren gemäss entweder Anspruch 1 oder Anspruch 2, wobei der gesättigte aliphatische Monoalkohol Cetylalkohol ist.

4. Verfahren gemäss einem der Ansprüche 1 bis 3, wobei das Gleitmittel weiterhin 1 bis 10 Gew.%, bezogen auf das Gesamtgewicht des Gleitmittels, Polybuten, Petroljelly oder Butylstearat enthält.

5. Verwendung eines gesättigten aliphatischen Monoalkohols mit 14 bis 18 Kohlenstoffatomen als festes Gleitmittel bei der Kaltbearbeitung eines Metallwerkstücks, welches von der Oberfläche des Metalls durch Erhitzen ohne Fleckenbildung entfernt wird.

6. Verwendung gemäss Anspruch 5, wobei der gesättigte aliphatische Monoalkohol Cetylalkohol ist.

7. Verwendung gemäss entweder Anspruch 5 oder Anspruch 6, wobei das Gleitmittel auch 1 bis 10 Gew.%, bezogen auf das Gesamtgewicht des Gleitmittels, Polybuten, Petroljelly oder Butylstearat enthält.

8. Verwendung einer Zusammensetzung, umfassend eine Lösung eines gesättigten aliphatischen Monoalkohols mit 14 bis 18 Kohlenstoffatomen in einem inerten flüchtigen, organischen Feststoff, als Gleitmittelfilm-bildendes Mittel bei der Kaltbearbeitung eines Metallwerkstücks, um einen Film von einem festen C₁₄₋₁₈-gesättigten aliphatischen Monoalkohol-Gleitmittel auf der Werkstückoberfläche zu bilden, welcher von der Metalloberfläche durch Erhitzen ohne Fleckenbildung entfernt wird.

9. Verwendung gemäss Anspruch 8, wobei der gesättigte aliphatische Monoalkohol Cetylalkohol ist.

10. Verwendung gemäss entweder Anspruch 8 oder Anspruch 9, wobei das inerte flüchtige, organische Lösungsmittel ausgewählt wird aus Trichlorethylen und 1,1,1-Trichlorethan.

11. Verwendung gemäss einem der Ansprüche 8 bis 10, wobei die Lösung etwa 10 Gew.% des gesättigten aliphatischen Monoalkohols enthält.

12. Verwendung gemäss einem der Ansprüche 8 bis 11, wobei die Lösung zusätzlich ein Material, ausgewählt aus Polybuten, Petroljelly und Butylstearat, in einer Menge von 1 bis 10 Gew.% in bezug auf das vereinte Gewicht des gesättigten aliphatischen Monoalkohols und dieses Materials, enthält.

13. Verwendung gemäss einem der Ansprüche 5 bis 12, wobei das Metallwerkstück aus Aluminium oder einer Aluminiumlegierung gebildet wird.

14. Verwendung gemäss einem der Ansprüche 5 bis 13, wobei das Metallwerkstück in Form einer Röhre für einen Kaltziehvorgang ausgewählt wird.

## Revendications

1. Un procédé pour le façonnage froid d'une pièce métallique à usiner, comportant le fait de prévoir sur la surface de la pièce à usiner devant être soumise à la formation d'un film de lubrifiant, de soumettre la pièce à usiner à une opération de formage et d'élimincr le film de lubrifiant de la surface du métal, caractérisé en ce que le film de lubrifiant comporte un film solide d'un alcool aliphatique monohydrique saturé, ayant de 14 à 18 atomes de carbone, et en ce que le film de lubrifiant est éliminé de la surface métallique sans provoquer de salissure en y appliquant de la chaleur.

2. Un procédé selon la revendication 1, dans lequel le film solide de lubrifiant est amené à s'écouler sur la surface métallique en un point où la pression, due à l'opération de formage est appliquée.

3. Un procédé selon la revendication 1 ou la revendication 2, l'alcool aliphatique saturé monohydrique est l'alcool cétylique.

4. Un procédé selon l'une quelconque des revendications 1 à 3, dans lequel le lubrifiant renferme en outre de 1 à 10% en poids, par rapport au poids total de lubrifiant, d'un polybutène de pétrolatum ou de stéarate de butyle.

5. L'utilisation d'un alcool aliphatique saturé monohydrique, ayant de 14 à 18 atomes de carbone en tant que lubrifiant solide dans le façonnage à froid d'une pièce métallique à usiner, éliminée de la surface du métal par chauffage sans salissure.

6. L'utilisation selon la revendication 5, dans laquelle l'alcool aliphatique saturé monohydrique est l'alcool cétylique.

7. L'utilisation selon l'une quelconque des revendications 5 ou 6, dans laquelle le lubrifiant renferme également de 1 à 10% en poids, par rapport au poids total du lubrifiant, d'un polybutène, de pétrolatum ou de stéarate de butyle.

8. L'utilisation d'une composition comportant une solution d'un alcool aliphatique saturé monohydrique, ayant de 14 à 18 atomes de carbone, dans un solvant organique, inerte et volatil, en tant qu'agent formateur de film lubrifiant dans le façonnage à froid d'une pièce métallique à usiner afin de former un film d'un lubrifiant à base d'un alcool aliphatique saturé en C₁₄ à C₁₈, monohydrique sur la surface de la pièce à usiner, éliminé de la surface du métal par chauffage sans laisser de salissure.

9. L'utilisation selon la revendication 8, dans laquelle l'alcool aliphatique saturé, monohydrique est l'alcool cétylique.

10. L'utilisation selon l'une quelconque des revendications 8 ou 9, dans laquelle le solvant organique, volatil et inerte est choisi parmi le trichloroéthylène et le 1,1,1-trichloréthane.

11. L'utilisation selon l'une quelconque des revendications 8 à 10, dans laquelle la solution renferme environ 10% en poids d'alcool aliphatique saturé, monohydrique.

12. L'utilisation selon l'une quelconque des revendications 8 à 11, dans laquelle la solution renferme en outre un matériau choisi parmi un polybutène, du pétrolatum et du stéarate de butyle en une quantité de 1 à 10% en poids en se basant sur le poids combiné de l'alcool aliphatique saturé monohydrique et dudit matériau.

13. L'utilisation selon l'une quelconque des revendications 5 à 12, dans laquelle la pièce métallique à usiner est formée d'aluminium ou d'un alliage d'aluminium.

14. L'utilisation selon l'une quelconque des revendications 5 à 13, dans laquelle une pièce métallique à usiner sous forme d'un tube est choisie pour une opération d'étiragc à froid.
